

Nov. 28, 1939.

M. F. PERKINS ET AL

2,181,148

PROCESS AND APPARATUS FOR PRODUCING ZINC

Filed Oct. 19, 1937

3 Sheets-Sheet 1

*Fig. 1*



*Fig. 3*



*Fig. 2*



INVENTORS  
Melville F. Perkins  
By Roland G. Crane  
James A. Kunk  
ATTORNEY

Nov. 28, 1939.

M. F. PERKINS ET AL

2,181,148

PROCESS AND APPARATUS FOR PRODUCING ZINC

Filed Oct. 19, 1937

3 Sheets-Sheet 2



Fig. 4

INVENTORS  
Melville F. Perkins  
BY Roland G. Crane

James H. Reid  
ATTORNEY

Nov. 28, 1939.

M. F. PERKINS ET AL

2,181,148

PROCESS AND APPARATUS FOR PRODUCING ZINC

Filed Oct. 19, 1937

3 Sheets-Sheet 3

Fig. 5



Fig. 6



INVENTORS  
Melville F. Perkins  
BY Roland G. Crane  
James K. Kent  
ATTORNEY

## UNITED STATES PATENT OFFICE

2,181,148

PROCESS AND APPARATUS FOR PRODUCING  
ZINC

Melville F. Perkins and Roland G. Crane, Woodbridge, N. J., assignors to American Smelting and Refining Company, New York, N. Y., a corporation of New Jersey

Application October 19, 1937, Serial No. 169,773

15 Claims. (Cl. 75—26)

This invention relates to the art of reducing oxidized ores or calcines of metals whose reduction temperatures exceed the boiling points of the particular metals. As zinc is the outstanding example of such a metal, the invention will be described with particular reference thereto.

It is known to produce zinc by introducing finely-divided zinc ore or calcine and carbonaceous reducing agent into a retort maintained at zinc reduction temperatures whereby the zinc content of the open, non-compacted charge is reduced practically instantaneously in suspension to vapor, passing the zinc vapor and accompanying gases through a bed of incandescent coke to separate out the dust carried by the gases and to convert any carbon dioxide to carbon monoxide, and treating the emerging vapors to recover the zinc content, e. g., by condensation. Such process is disclosed in United States Letters Patent No. 2,096,779 granted October 26, 1937 to George P. Bartholomew and Edward P. Fleming.

The procedure just described may be aptly termed a "flash" reduction and the acceptable theory of operation divides the actual reduction of the ore or calcine into two steps, the first of which is expressed by the reaction



and the second by the reaction



Various data indicate that Reaction 1 proceeds much faster than does Reaction 2 so that for successful flash reduction, conditions must be such that Reaction 2 will proceed with sufficient speed to maintain an ample concentration of carbon monoxide in the reduction unit to permit reduction of substantially all of the zinc oxide in accordance with Reaction 1 before the particles pass from the reduction zone.

Among the various factors to be considered in the balancing of conditions to assure the proper speed of Reaction 2 for maximum zinc reduction are: the height of the flash shaft, the temperature of the reduction zone of the flash shaft, the degree of preheat of the charge, the reactivity of the carbonaceous component of the charge—tests show powdered charcoal to be twice as reactive in the flash shaft as is ordinary metallurgical coke, the ratio of carbon to ore or calcine in the charge, the degree of pulverization or subdivision of the carbonaceous component of the charge, and the use of catalytic agents to speed the producer gas reaction—tests show that the addition of small amounts of soda ash, say under

1%, to the carbonaceous component of the charge increases the rate at which carbon dioxide is reduced in accordance with Equation 2 and thus made available for the reduction of the zinc component of the charge in accordance with Equation 1.

From what has just been said, it will be apparent that, viewed from the standpoint of securing maximum efficiency in the zinc reduction step, the zinc vapors withdrawn from the flash shaft and passed into the coke filter should contain no appreciable amount of carbon dioxide. Unfortunately, however, the zinc vapor and carbon monoxide leaving the flash column are accompanied by suspended particles of carbon entrained in the vapors and the burden which this places on the filtering medium presents a very real obstacle to successful continuous operation of the flash reduction unit as a whole. Further, it is not practicable to eliminate the dust by increasing the size of the particles of ore or reducing fuel because of the adverse effect on reduction and while clogging of the filtering medium may be mitigated by using coarser coke fragments, say of two-inch size, the advantage is nullified by the detrimental effect on condensation occasioned by suspensoids passing through into the condenser.

In order, therefore, to alleviate the adverse influence of the dust, it has been proposed to continuously renew the filtering medium (as by confining same as an upright column and withdrawing coke from the bottom while adding additional coke at the top) while passing the zinc vapors therethrough thereby removing the suspensoids from the vapor stream and preventing clogging of the medium. While such procedure is wholly operable, it presents several disadvantages among which are the relatively large amounts of coke required to be put through the column to maintain it in an open condition, the difficulty of maintaining the filtering medium at a constant temperature due to the more or less continuous changing or renewal of the medium itself, and the tendency for a portion of the zinc to condense in that part of the medium which lies outside of the direct flow of the vapors thus either resulting in that portion of the zinc passing out with the coke residues or requiring some corrective measure, such as provision of a suitable draft through that part of the filtering medium, to prevent such condensation.

The present invention provides certain improvements in the flash reduction process and apparatus therefor which avoid clogging or

choking of the coke column while permitting the use of a stationary coke bed with its attendant advantages and at the same time maintaining the reduction and condensation operations at their 5 respective maximum efficiencies.

In short the invention may be said to be largely based upon the discovery that improved results are obtained when the vapors withdrawn from the flash reducer are subsequently treated, 10 not merely by a process of filtration, but, by a very definite and positive process of conditioning based upon oxidation of carbon to carbon monoxide by the producer gas reaction,  $\text{CO}_2 + \text{C} \rightarrow 2\text{CO}$ , or otherwise.

15 Essentially this conditioning process consists in imparting to or establishing in the vapors an oxidizing gas content sufficiently in stoichiometrical excess of the carbon in the particles entrained in the vapors to consume enough of the 20 incandescent coke bed through which the vapors pass to render the bed self-cleaning thereby permitting the use, if desired, of a stationary coke bed with its many attendant advantages.

While it is preferred to employ carbon dioxide 25 as the oxidizing gas, the conditioning process is not limited to its use. For example, air may be employed. Also, a choice exists as to the manner in which the requisite oxidizing gas content is supplied to the vapors. Thus, it may be introduced 30 into the vapor stream as the latter emerges from the flash reducer with its burden of entrained particles; it may be introduced in the vicinity of the vapor entrance to the column or bed of incandescent coke and, particularly if 35 carbon dioxide is the gas used, it may be established in the vapors before they leave the flash reducer by simple regulation of the ratio of powdered coke to ore charged to the flash reducer shaft. In the latter case, care should be exercised not to impair reduction efficiency—if the 40 residue at the bottom of the reducer shaft tends to become fusible or of a slaggy nature, sufficient coarse-sized coke particles may be incorporated in the charge to maintain the residue in good 45 condition for ready withdrawal from the shaft as a pulverulent material. However, the residue may be withdrawn as a slag, if desired.

Although the novel features which are believed 50 to be characteristic of this invention will be particularly pointed out in the claims appended hereto, the invention itself, as to its objects and advantages, and the manner in which it may be carried out, may be better understood by referring to the following description taken in connection with the accompanying drawings forming 55 a part thereof, in which—

Fig. 1 is a view of a flash reduction unit according to the invention, the feeding mechanism and condenser being diagrammatically indicated 60 and the remainder of the unit being shown in vertical section;

Fig. 2 is an enlarged view of a portion of the apparatus shown in Fig. 1;

Fig. 3 is a cross-section taken on the line 3—3 65 of Fig. 1;

Fig. 4 is a fragmentary sectional elevation of a modification of the apparatus shown in Figs. 1—3;

Fig. 5 is a plan view of the feeding mechanism diagrammatically indicated in Fig. 1;

70 Fig. 6 is a sectional elevation taken on the line 6—6 of Fig. 5.

Like reference characters denote like parts in the several figures of the drawings.

Referring to the drawings, 10 represents generally the feeding mechanism for delivering the

charge to the flash reducer 12 from which the vapors are conducted through coke chamber 14 to condenser 16.

Referring particularly to Figs. 5 and 6, the feeding mechanism 10 is shown comprising a hopper 20 leading into housing 22 in which is screw conveyor 24 driven by motor 26 via speed reducer 28. The housing 22 opens into heating chamber 30 defined by muffle 32 which is surrounded by housing 34 defining combustion chamber 36 to which heat may be supplied by fuel burners or electric heating means not shown. Heating chamber 30 is provided with a gas outlet 38 and a thermocouple tube 40 extends through muffle 32 and housing 34 to the heating chamber 30. A pipe section 42 provided with flanged ends 44 and 46 connects muffle 32 with elbow 48, the latter in turn being secured to and opening into refractory discharge tube 50. Elbow 40 is provided with a sloping or tapered intake portion 52 above which is a rotative feeder 54 provided with blades or vanes 56, the feeder being driven by motor 58 via speed reducer 60. A punching or cleaning rod 62 with annular flange 64 is positioned at the top of elbow 48, the rod 62 passing through removable cap 66.

Referring now to Figs. 1, 2 and 3, the flash reducer 12 is shown comprising a vertically disposed column or shaft 70 of silicon carbide or other refractory material positioned in a combustion chamber 72 defined by heat insulating housing 74 surrounded by steel shell 76. A flue 78 is provided for the combustion chamber 72 to which heat is supplied by burners 80 which are preferably arranged to open tangentially into the combustion chamber and thereby impart a whirling motion to the flames and hot combustion products around the tubular shaft 70. Spaced supports 82 are provided for intermediately securing the shaft 70, the latter being supported at its bottom by a seat 84 in refractory housing 74 while its top is surrounded by the housing which converges at that point. The reducing unit is shown as supported by I-beams 86 resting on foundation 88. From the bottom of shaft 70, a conduit 90 leads to residue pit 92 provided with clean-out door 94.

In the construction illustrated in Figs. 1 and 2, a refractory conduit 96 provided with inlet 98 for carbon dioxide or other oxidizing gas leads to coke chamber 14, the latter in this case comprising a refractory column 100 positioned in a chamber 102 defined by a refractory housing 104 and heat insulation 106 and to which heat is supplied by burner 108 and hot gases from chamber 12 which pass around conduit 96 to chamber 102. A flue 109 is provided for chamber 102.

As clearly shown in Fig. 2, the conduit 96 is joined to shaft 70 by a butt-joint 110 while its other end is received in a cradle 112 which holds it in registry with the inlet port 114 at the bottom of the column 100. The detail of the latter mounting is shown in Fig. 3. Opposite inlet port 114 is an opening 116 affording access to the bottom of the coke column, said opening being normally closed by plug 118 which may be covered with removable cement or the like 120. An inclined grate 122 supports a bed of coke or other carboniferous material 124 in column 100, the top of said column being sealed by refractory cover 126. Vapor conduit 128 leads from the top of column 100 to condenser 16, an opening 130 normally closed by removable plug 132 being provided in the top of the column 100 opposite conduit 128. The coke chamber 14 and condenser 76

16 are shown supported independently of the flash reducer 12 by I-beams 134 and 136, respectively.

5 In the modification shown in Fig. 4, the reducer column is shown made up of refractory sections 138, the uppermost of which projects through an expansion slip-joint 140 into a header comprising a shell 142 and pipe 144 defining a combustion chamber 146 and resting on a base 10 147, which like the shell and pipe, is of suitable refractory material. The combustion space is continued around conduit 96 and coke column 100. Also in Fig. 4, one end of conduit 96 rests 15 on the top of pipe 144, the remaining space being bricked up and the conduit cemented in place while the other end engages a socket 148 on the bottom of the coke column.

15 In the coke column shown in Fig. 4, the sloping grate 122 of Figs. 1 and 2 has been replaced by a horizontal grate 150 which is positioned up 20 in the column a substantial distance from the bottom and supported by a body of refractory brick checkerwork 152. Suitable openings 154 and 156 which are normally closed by plugs 158 and 160, respectively, are provided.

25 The condenser 16a is shown provided with baffles 162 for imparting a tortuous path of flow to the vapors entering from conduit 128a. An opening normally closed by plug 164 permits access to conduit 128a for cleaning and a tap hole 166 is provided for withdrawing liquid zinc. An auxiliary condenser 168 provided with vent 170 and clean-out 172 is connected to the main condenser 16a by conduit 174.

30 Employing the apparatus hereinbefore described, the flash reduction process may be conducted as follows: a finely divided charge comprising a solid carbonaceous reducing agent and oxidized zinciferous material is fed to the hopper 20 from whence it passes by screw conveyor 24 into the muffle 32 where it is preheated. The charge may appropriately consist of flash roasted zinc calcine and coke dust with a majority of the particles minus 200-mesh. With the present 35 invention the amount of powdered coke or other carbonaceous material used in the charge may be varied within wide limits without impairing the efficiency of the operation.

35 The feeder 54 stirs up the charge and delivers it evenly to the tube 50 through which it drops by gravity into the reducer shaft 70 which has been previously brought to zinc reduction temperature by the combustion of fuel supplied by burners 80. In shaft 70 the oxidized zinciferous material is reduced practically instantaneously and zinc vapors together with the gaseous products of reaction, and suspensoids pass into refractory conduit 96.

40 It will be recalled that reduction of the zinc is accomplished by carbon monoxide according to Reaction 1 and that an ample concentration of carbon monoxide is maintained according to Equation 2 by reason of the presence of carbon in the charge. Accordingly, if sufficient coke is used so that the vapors entering conduit 96 contain very little carbon dioxide, complete reduction is assured. However, the carbonaceous suspensoids entrained in the vapor if permitted to remain as such would collect in the interstitial 45 spaces of the non-moving coke in the coke column and prevent further flow of vapor through the coke thereby terminating the entire operation in a short time.

45 In accordance with the modification of the apparatus of the invention illustrated in Figs. 1

5 and 2, carbon dioxide or other oxidizing gas is introduced into conduit 96 through inlet 98 in an amount sufficient to convert the carbon of the entrained particles to carbon monoxide and to consume sufficient coke in the column 100 to 10 render said coke column continuously self-operating. The gas introduced through inlet 98 is preferably of the same, or of approximately the same, temperature as the vapors entering conduit 96 from the flash shaft. Thus conditioned, 15 the vapors pass upwardly through the coke column so that only pure zinc vapor and carbon monoxide pass to the condenser 16. Coke is supplied to column 100, intermittently as needed, 20 through refractory cover 126.

25 As previously brought out the present invention also contemplates other methods of conditioning the vapor and operating the coke column as a reactor to maintain same continuously self-operating by automatically keeping open the interstitial spaces between the units of the coke aggregate. Thus a small amount of air can be introduced at the base of the coke column and the entrained carbonaceous suspensoids in the vapors eliminated at that point. Satisfactory results have been obtained in actual practise without the introduction of extraneous gas by simply supplying the vapors from the flash shaft itself to the conduit 96 with a sufficient carbon dioxide content to satisfy the necessary chemical 30 reactions. The operation has been conducted in this manner so efficiently that less than 1% to 2% of the zinc content of the charge was found in the residues at the base of the flash shaft.

35 In passing from the flash shaft to the base of the coke column, the velocity of the vapors is somewhat diminished in the closure at the base of the coke column thereby allowing the coarser particles to settle and the reaction of the oxidizing gas upon the carbonaceous suspensoids to 40 proceed. The vapors then pass through the grate 122 as shown in Figs. 1 or 2 or through the checker brickwork 152 as shown in Fig. 4 into the coke or reactor column, the baffles promoting turbulent gas flow and retardation of the flight 45 of any fine suspensoids in the vapor stream.

45 Among the many advantages attending the use of the invention, the most important may be said to be the truly continuous and efficient operation of the flesh reduction process which it provides. 50 With the invention it is possible to operate the process indefinitely without the shut-downs and costly delays which inevitably accompany choking or clogging of the coke bed and while the benefits are more pronounced when using a stationary coke bed, it will be understood that the invention may be employed in conjunction with a moving coke column.

55 While the invention has been described with reference to the production of zinc, it will be apparent that it may be applied to the treatment of other artificial or natural oxidic ores where, as with zinc, the reduced metal is in the vapor state.

60 What is claimed is:

65 1. The process for treating oxidized zinciferous material which comprises charging such material and solid carboniferous material, both materials being in a fine state of subdivision, into a retort wherein the zinciferous material is reduced in suspension, passing the products of reaction as a 70 stream to an incandescent carboniferous bed, supplying an oxidizing gas to the stream in amount sufficient to oxidize the carboniferous suspensoids entrained in said stream and render the carboniferous bed self-cleaning, passing the stream 75

through said bed and recovering zinc from the gases emerging therefrom.

2. The process for treating oxidic ore of a metal requiring a temperature above its boiling point for successful reduction which comprises charging such ore and a carbonaceous reducing agent to a substantially vertically-disposed retort maintained at a temperature conducive to reduction of the ore, both ore and reducing agent 10 being introduced to the retort in a sufficiently fine state so that reduction is accomplished practically instantaneously in suspension, causing the products of reaction to flow as a stream to and through a bed of incandescent carbonaceous material, conditioning the stream with an oxidizing gas to consume carbonaceous suspensoids and render said bed self-cleaning, withdrawing the conditioned vapor from said bed and recovering metal from said vapor.

20 3. The process for treating oxidized zinciferous material which comprises passing an intimate, finely-divided mixture of said zinciferous material and carboniferous reducing agent into a substantially vertically-disposed retort, effecting a 25 substantially instantaneous reduction of the zinciferous material in suspension, passing the products of reaction as a vapor stream through an incandescent carboniferous bed, maintaining a substantial amount of carbon dioxide in the 30 said vaporous reaction products, causing said carbon dioxide to react upon carboniferous suspensoids entrapped in the vapor stream thereby enriching said stream in carbon monoxide, completing the reduction of residual carbon dioxide 35 to carbon monoxide in the carboniferous bed thereby preventing choking of the said bed with suspensoids in the vapor stream, and condensing zinc from the vapors emerging from the said carboniferous bed.

40 4. The process for treating oxidized zinciferous ores and calcines which comprises passing an intimate, finely-divided charge of such zinciferous material and carboniferous reducing agent into a substantially vertically-disposed retort and effecting substantially instantaneous vaporization 45 of the zinc therein, providing a substantial amount of carbon dioxide in the vapor stream emerging from the retort, said carbon dioxide being in stoichiometrical excess of carbon entrained in the stream, producing a reaction between the carbon dioxide and carboniferous suspensoids in the vapor stream, said reaction being caused to proceed intermediate the retort and a bed of incandescent coke to and through which 50 the stream is next conducted, reducing in the coke bed any unreduced zinciferous suspensoids present in the vapor stream and also reducing to carbon monoxide any carbon dioxide remaining in said stream thereby rendering the coke bed 55 self-cleaning and the zinciferous vapor stream substantially free from carbon dioxide and suspensoids, and condensing zinc from the thus purified vapor stream.

5. The process for producing zinc which comprises passing an intimate, finely-divided mixture of oxidized zinciferous material and carboniferous reducing agent into a substantially vertically-disposed retort heated to a temperature conducive of zinc reduction, withdrawing the 60 products of reaction from the retort as a vapor stream, establishing a substantial amount of carbon dioxide in said vapor stream, imparting turbulence of flow and heat for reaction to said vapor stream for a period sufficing to reduce 70 zinciferous suspensoids and carbonaceous sus-

75 pensoids to zinc vapor and carbon monoxide, respectively, then passing said stream into a bed of incandescent carbonaceous material wherein any carbon dioxide remaining in the stream is reduced to carbon monoxide at the expense of a small amount of the carbon of said bed and the interstitial spaces of the aggregate are maintained in an open state for the passage of the vapor stream therethrough, and condensing zinc from the conditioned stream emerging from the 10 carboniferous bed.

6. The process for treating oxidized zinciferous material which comprises reducing same in suspension with such a kind and amount of carbonaceous reducing agent as to impart a substantial content of carbon dioxide to the vapor withdrawn from the reducer, passing the vapor to and through an incandescent bed of carbonaceous reducing agent, retarding the flow of vapor intermediate the reducer and bed sufficiently to permit oxidation by the carbon dioxide of carbonaceous suspensoids entrained in the vapor and recovering zinc from the vapor which has passed through said bed.

7. In the process for producing zinc by flash 25 reducing the zinc in a charge of oxidized ore or calcine and coke or other carboniferous reducing agent, passing the products of reaction through an incandescent bed of carboniferous reducing agent and recovering zinc from the emerging vapors, the improvements consisting in utilizing sufficient coarse coke in the charge to prevent slagging of the reduction residue and maintaining a carbon dioxide content in the 30 products of reaction as same pass from the flash reducer to said incandescent bed that is in stoichiometrical excess of the carbon content of 35 said products of reaction.

8. In the flash reduction of oxidized zinciferous materials with a carbonaceous reducing agent following which the vapors are conducted through a carboniferous bed maintained at a temperature above that at which the zinc would condense, that improvement which consists in conducting the reduction in such a manner that the zincy vapors withdrawn from the reducer contain a sufficient amount of carbon dioxide in stoichiometrical excess of carbon entrained in the vapors to render the carboniferous bed non-clogging and maintain it continuously open 45 to the passage of vapors therethrough.

9. Apparatus for treating oxidized ores or calcines comprising the combination with a flash reduction shaft furnace, and a bed of carboniferous material, of means for conveying vapors from said furnace into said bed, and means for introducing gas into said vapors subsequent to their withdrawal from the reduction shaft but prior to their entrance into the carboniferous bed.

10. Apparatus for treating oxidized ores or calcines comprising the combination with a flash reduction retort, a confined bed of carbonaceous material and a conduit connecting the vapor outlet of said retort to the vapor inlet of said bed, of means associated with said conduit intermediate the retort and bed retarding the flow of vapors before same enter said bed.

11. Apparatus for reducing finely divided oxidized ores and calcines and recovering metal therefrom comprising a vertically disposed retort, means for externally heating the retort to reduction temperatures, a closure, a duct interconnecting said retort and closure for leading gaseous materials from the retort to the said closure, a grate member in said closure support- 70 75 75

ing therein a bed of carboniferous material and so positioned that vapors emerging from said duct pass through said grate before entering said bed, means for externally heating said bed, means 5 intermediate the retort and the bed for retarding flow of gaseous reaction products from the retort to the bed, and condensing instrumentalities interconnected with the said closure containing the bed for effecting condensation of the metallic components of the reaction products issuing from the said closure.

12. Apparatus for treating finely divided oxidized materials, such as oxidized zinciferous ores or calcines, comprising a vertically disposed retort, means for externally heating the retort, a closure, a duct interconnecting the retort and the bottom of said closure for passing gaseous materials from the former to the latter, a grate in said closure adapted to support therein a bed 20 of carboniferous material of considerable thickness at a point substantially above the opening of said duct into the closure, means for externally heating the said bed, means defining a reaction chamber intermediate the retort and the bed for retarding the velocity of gaseous reaction products flowing from the retort to the bed, and condensing instrumentalities interconnected with the said closure containing the bed for effecting condensation of the metallic components of the reaction products issuing from 25 the said closure.

13. Apparatus for the reduction of oxidic ores and calcines comprising the combination with a vertically disposed retort and heating means therefor, of mechanism for feeding a finely divided charge to the retort, said mechanism comprising an enclosed conduit, means for introducing a charge of the material to be reduced into said conduit, means operating through said conduit for conveying the charge therethrough, heating instrumentalities in said conduit for preheating the charge as it is conveyed therethrough,

and means engaging the said charge as it emerges from said conduit and uniformly feeding the charge into the retort.

14. Apparatus for reducing finely divided oxidized materials comprising the combination with a substantially vertically disposed, externally-heated retort, of feeding mechanism for introducing a charge of such material into the retort, said mechanism comprising a closed conduit, a hopper for delivering materials into said conduit, a screw conveyor operating in said conduit, heating means for the conduit for preheating the charge of materials being conveyed therethrough, feeding instrumentalities intermediate said screw conveyor and the retort for receiving the charge as it leaves the screw conveyor and uniformly feeding the charge into said retort without substantial cooling of the preheated charge and cleaning means for maintaining the entrance to the retort open.

15. Apparatus for reducing finely divided oxidized ores and calcines comprising the combination with an externally heated, substantially vertically disposed retort, of feeding mechanism for the said retort for feeding a charge of materials uniformly therethrough, the said feeding mechanism comprising a closed conduit, a hopper for delivering a charge of materials into the conduit from a suitable source thereof, a screw conveyor operating in the conduit, an upwardly flaring connecting delivery section between the said conduit and the retort, a heating muffle in the said conduit for preheating the charge of material being conveyed therethrough, and a rotary feeding device in the upper part of the 35 said flaring, connecting delivery section for receiving preheated material from the screw conveyor and for uniformly feeding the said material into the said connecting delivery section and retort.

MELVILLE F. PERKINS.  
ROLAND G. CRANE.